

Dec. 16, 1930.

C. B. KINGSLEY

1,785,264

METHOD OF AND APPARATUS FOR ANNEALING MATERIALS

Filed March 8, 1927

3 Sheets-Sheet 1

Fig. 1



INVENTOR

Charles B. Kingsley  
BY  
Cooper, Penick & Denham  
HIS ATTORNEY

Dec. 16, 1930.

C. B. KINGSLEY

1,785,264

METHOD OF AND APPARATUS FOR ANNEALING MATERIALS

Filed March 3, 1927

3 Sheets-Sheet 2



Fig. 2

INVENTOR  
*Charles B. Kingsley*  
BY  
*Cooper, Herr & Dunham*  
HIS ATTORNEY

Dec. 16, 1930.

C. B. KINGSLEY

1,785,264

METHOD OF AND APPARATUS FOR ANNEALING MATERIALS

Filed March 8, 1927

3 Sheets-Sheet 3

Fig. 3



Fig. 4



Fig. 5



Fig. 6



INVENTOR

Charles B. Kingsley  
BY  
Cooper, Kerr & Dunham  
HIS ATTORNEYS

## UNITED STATES PATENT OFFICE

CHARLES B. KINGSLEY, OF CLAIRTON, PENNSYLVANIA, ASSIGNOR TO MISSISSIPPI  
GLASS COMPANY, A CORPORATION OF NEW YORK

## METHOD OF AND APPARATUS FOR ANNEALING MATERIALS

Application filed March 8, 1927. Serial No. 173,675.

The present invention relates to methods of and apparatus for annealing materials with special application to the continuous annealing of sheet glass.

5 The invention comprises new and novel methods of operating material-annealing apparatus and new and novel constructions of material-annealing apparatus hereinafter described and more particularly set forth in the 10 claims.

In the accompanying drawings I have shown for purpose of illustration a form of apparatus for practicing my invention in which

15 Figure 1 is a vertical section of one form of material-treating apparatus for annealing substances according to my new methods,

20 Figure 2 is a sectional view of the apparatus of Figure 1 and taken along line A—A thereof with the enclosing side wall broken away to show the arrangement of interior parts more clearly, and

25 Figures 3, 4, 5 and 6, show modified forms of my invention.

30 In the drawings the apparatus comprises a structure 2 having bottom, side walls and top as shown in section in Figure 1 with a system of live rolls 3, 3, which pass through the side walls 2 and find support and contact 35 with power actuating mechanism on either side of the structure, outside of the side walls 2 all of which is found in the apparatus as practiced in the art at the present time.

35 In the continuous annealing of a continuous formed sheet of glass I find it of advantage to adjustably suspend an inside horizontal flat or curved curtain or cover 4 of blocks of clay or other suitable material as shown in cross section in Figures 1 and 4, 40 and in longitudinal section, in part, in Figure 2, along the length of the annealing apparatus and in the space C between the rolls 3, 3, and the top wall of the apparatus.

45 For the raising and lowering of this horizontal curtain 4 suitable mechanical appliances are provided outside and above the enclosing structure 2 as indicated in Figure 1 comprising supporting screw stem hangers 5, 5, gear nuts 6, 6, operating worms 7, 7, and 50 operating shafts 8, 8.

In operating annealing apparatus of the indicated type without the special suspended horizontal curtain it has been found difficult and often impossible to control the air currents throughout the large cross section 55 of the enclosed space and inequalities in temperatures of the sheet take place, causing warping, splitting and general objectionable results, and it is the purpose of my invention to so protect and confine the continuous sheet 60 of glass shown at 9, being carried forward on the live rolls 3, that the required control of temperatures is possible for a proper annealing and cooling of the sheet to insure 65 a properly annealed and flat sheet, and thus prevent splits and breaks in the sheet due to 70 improper cooling.

In the operation of my annealing equipment the vertical adjustment of the hanging 75 horizontal curtain is essential as it is desirable to have it supported close to the sheet of glass so that the vertical sides of the curtain 80 4 may close in over the ends of the live rolls and prevent air currents from circulating under the curtain at this point, the curtain in 85 the lowered position as shown on the drawings forming a shallow flat or curved arch in which the tops of the rolls operate and through which they carry the sheet of glass and providing additional mass along the sensitive edge where otherwise cooling takes 90 place more rapidly than in the center of the sheet and thus I promote and obtain an equalized cooling of the sheet as a whole.

95 While a function of the horizontal curtain 85 is to stop air currents causing inequalities in temperature in the zone through which the glass sheet is passing an important factor is that the mass or material comprising the horizontal curtain absorbs the radiated heat from 90 the sheet of glass and because of its greater mass will not suffer local or zone changes in its temperature due to the circulating air currents in the larger chamber C caused by radiations from the enclosing surfaces of 95 chamber C, and the heat of the larger mass as furnished by the horizontal curtain 4 provides a uniform temperature across the sheet at any particular point or cross section and a gradual change in temperature longitudinally 100

of the horizontal curtain is obtained. The general heating or cooling of the main chamber C is obtained by adding heat by such means as gas flames, the latent heat of the entering sheet of glass and the controlled radiation of heat from the enclosing walls 2 of chamber C along the length thereof, as is known in the art.

The utilization of a vertically adjustable horizontal curtain 4 is of value in the continuous process of making sheet glass in two ways, i. e.: When the operation of making continuous sheet glass begins there is often a rough, lumpy surface, also elevated edges and projecting points so that it will be desirable to give additional clearance above the rolls 3 for the passage of the head end of the sheet. As the desired initial temperatures of the zones making up the total longitudinal dimension of chamber C will have been obtained before the entry of the hot sheet of glass, it is possible to have the horizontal curtain 4 in an elevated position for any desired clearances above the rolls 3 as an interval of time elapses between the entry of the sheet and the critical disturbance of desired temperature conditions initially established in which time the horizontal curtain 4 may be lowered to its operating position.

The second advantage in having a movable horizontal curtain 4 is that as the cooler zones in chamber C are reached by the advancing sheet of glass additional cooling effect may be obtained by increasing the distance of the horizontal curtain from the sheet.

To be able to establish varying operating distances between the horizontal curtain 4 and the sheet of moving glass or rolls 3 will also be a desirable feature when various thicknesses of sheet glass are to be annealed, as the latent heat of the sheet to be dissipated varies and the rate of travel of the sheet through the annealing chamber changes and a flexible control of the temperature in the annealing chamber is desired.

The horizontal openings between sections of the curtain 4 are closed by tile 6 or other suitable material to shut off air currents at these points, and the various sections along the length of the curtain may be adjusted in any desirable variation of height with relation to each other and to the rolls 3, 3, and the curtain may be made of two longitudinal members 4 and 4a as shown in Figure 3, leaving an open space along the length thereof, and said opening may be left open, or closed with tile, as shown at 7 in said Figure 3, either wholly or partially along the length thereof to meet the needs of service, as desired.

In some instances it may be desired to vary the distance of the various sections along the length of the curtain with relation to the rolls 3, 3, and the construction shown in Figure 5 will permit of obtaining practically the widest variations desired. Here, the sides of

the curtain 4 are shown as separate members 4b, 4b, suspended in fixed position and to have sliding engagement with the edges of the curtain 4.

In other instances, it may be desired to protect only the edges of the glass sheet from too rapid cooling and the curtain 4 can then be constructed and mounted as shown in Figure 6, to secure equalized cooling of the sheet as a whole.

As a further description of the principle in the application of a suspended horizontal curtain to the annealing of continuous sheet glass a comparison of the physical action which takes place in the annealing of a continuous thin glass sheet and the annealing of a continuous thick sheet of glass may be used. In the annealing of thin sheet glass the latent heat of the sheet is easily dissipated and being of less mass, with a lesser total latent heat, it is both easier to add or subtract heat to or from it at local points or areas, or over its entire area than is possible in the case of a thick sheet which naturally carries a greater total latent heat because of its greater mass. This susceptibility of the thin sheet of glass makes it easily affected by inequalities in the temperature of the chamber C and as before stated local air currents have quick and detrimental effect on the sheet of glass and cause warping, venting and general breakage with unequal tempering or annealing of the sheet.

In the annealing of a continuous thick sheet of glass a greater range of temperature variations is possible because of the less sensitive nature of thick sheet due to its greater mass and consequent higher total latent heat contained, which in practice does not show the same tendency to warp, check or break in the process of annealing.

This invention takes advantage of this principle by adding to the heat retaining mass of the thin sheet, the heat retaining mass of the horizontal suspended curtain, which having been brought up to local temperatures established in the chamber C before the entry of the sheet of glass serves both as a reservoir and an absorber of heat and a less susceptible mass from which heat may be taken without the local differences suffered by a body of small mass as contained in a thin sheet of glass.

While the advantages of the horizontal suspended curtain are not so pronounced in its application to the annealing of heavy or thick continuous sheet glass, still its sluggish or slow response to quick or local changes in temperature in chamber C will aid in the more satisfactory and perfect annealing of the sheet and is equally desirable.

An advantage of great importance in this invention is that the latent heat of the continuous sheet of hot glass is conserved in the horizontal suspended curtain and will reduce materially the quantity of heat to be supplied.

or added to the chamber C if not under some conditions making the adding of additional heat unnecessary thereby working a desirable and beneficial saving in the cost of annealing.

5. I claim:

1. The method of annealing a continuously formed sheet of glass, comprising advancing the sheet of glass through an annealing chamber of fixed cross section, and controlling the 10 rate of cooling of the sheet of glass as it passes through said chamber by interposing between the upper surface of the sheet and the upper wall of said chamber a heat absorbing and heat retaining element without restricting the cross sectional area of the chamber.

2. The method of annealing a continuously formed sheet of glass, comprising advancing the sheet of glass through an annealing chamber of fixed cross section, and controlling the rate of cooling of said sheet through any cross sectional area of the chamber by interposing heat absorbing and retaining element intermediate the sheet and the top wall of 25 the chamber, said element serving to eliminate objectionable air currents around and about said sheet and limiting the cross sectional area only by its own cross sectional area.

3. In an apparatus for annealing a continuously formed sheet of glass, the combination comprising an open ended treating chamber of fixed cross section, means for conveying a sheet of glass through said chamber, and means for equalizing the distribution of 20 heat transfer in a sheet of glass at any cross section thereof, said means comprising a curtain of heat absorbing and retaining material disposed above the sheet of glass and 40 within said treating chamber, said curtain restricting the cross sectional area of said chamber only by its own cross section.

4. In an apparatus for annealing a continuously formed sheet of glass, the combination comprising an open ended treating chamber of fixed cross section, means for conveying a sheet of glass through said chamber, and a heat absorbing and heat retaining curtain disposed immediately above the sheet of 50 glass and away from the walls of said open ended chamber.

5. In an apparatus for annealing a continuously formed sheet of glass, the combination comprising an open ended treating chamber of fixed cross section, means for conveying a sheet of glass through said chamber, and means for eliminating objectionable air currents at the edges of the sheet of glass and 55 immediately above its upper surface, said means comprising a curtain of heat absorbing and retaining material spaced from the upper wall of said open ended chamber.

6. In an apparatus for annealing a continuously formed sheet of glass, the combination comprising an open ended treating chamber

of fixed cross section, means for conveying a continuous sheet of glass through said chamber, means for eliminating objectionable air currents around and about said sheet comprising a curtain of heat absorbing and retaining material interposed between the sheet and the upper wall of the chamber, said sheet restricting the cross sectional area of the chamber only by its own cross section, and means for regulating the position of the aforesaid means between the sheet and the upper wall of the oven.

In testimony whereof I hereto affix my signature.

CHARLES B. KINGSLEY.

80

85

90

95

100

105

110

115

120

125

130